

May 7, 1957

C. G. CHAMBERS ET AL

2,791,516

## ELECTROLESS PLATING

Filed Sept. 17, 1953



INVENTORS  
Clarence G. Chambers &  
Robert C. Spaulding  
BY  
*S. E. Ross*  
ATTORNEY

1

2,791,516

## ELECTROLESS PLATING

Clarence G. Chambers, Ypsilanti, and Robert A. Spaulding, Huntington Woods, Mich., assignors to General Motors Corporation, Detroit, Mich., a corporation of Delaware

Application September 17, 1953, Serial No. 380,858

9 Claims. (Cl. 117—102)

This invention relates to improvements in the deposition of metal from chemical reduction type plating solutions.

It is known that nickel and other metals can be deposited without the use of electrical current by immersing an article to be coated into an aqueous solution of a nickel or other metal salt and a reducing agent such as sodium hypophosphite or potassium hypophosphite. There are two types of such plating solutions, namely, alkaline and acid, of which the acid solution is generally better adapted for commercial plating operations. The plating by chemical reduction is usually conducted at an elevated temperature, typically about 90° C.

One of the difficulties heretofore encountered in the commercial adaptation of chemical reduction plating has been the inability to preclude deposition of metal on the plating equipment with the result that in many instances an undesirable metallic deposit is produced throughout the plating equipment. Not only does such a deposit deplete the metal content of the plating solution but it also impairs heat transfer and acts as a catalyst increasing the undesired deposition of metal.

The exact nature of the chemical plating reaction is not clearly understood at present. However, it has been observed that certain metals, such as lead, copper, brass or platinum which would not ordinarily be coated by the oxidation-reduction plating reaction, do become susceptible to being coated when, for example, momentarily brought in contact with aluminum or other reaction initiating material. Inasmuch as the exact nature of such an initiating reaction is not clearly understood the failure to control the deposition of nickel and other metals deposited by chemical reduction methods in certain cases is a serious problem even though the plating equipment is formed from a material which theoretically should not become coated during the plating reaction. The problem, of course, is even more serious in large scale reduction plating operations which employ plating tanks, piping and other equipment formed of metals, such as iron, steel, nickel, aluminum and alloys of these metals, which are readily coated with the metal being deposited.

A principal object of the present invention is to provide a chemical reduction plating process in which the aforementioned difficulties are minimized. A further object is the provision of an improved chemical reduction plating process. A still further object is the provision of an improved plating operation in which maintenance of proper solution concentration is facilitated while effectively controlling the metallic deposition. These and other objects and advantages of the invention will more fully appear from the following description taken in connection with the accompanying drawing which illustrates in schematic form apparatus for the operation of a chemical reduction plating process in accordance with the present invention.

Generally, we have discovered that undesirable metallic deposition throughout the plating equipment can effectively be minimized and precluded entirely in many

2

applications by constantly recirculating the plating solution and by quench cooling a portion of this solution from the high bath temperature required for optimum plating to a temperature at which little or no plating occurs and thereafter recirculating the cooled solution into the plating tank. By proper control, using this technique, sufficient plating solution is quenched to preclude metallic deposition throughout the equipment; yet an excessive amount of heat energy is not wasted in so doing.

10 In the drawing the single figure is a schematic diagram of apparatus used in performing the plating process.

For the continuous operation of a plating solution, quench cooled in accordance with the invention, the maintenance of proper solution concentration is contemplated by continuously or intermittently introducing into the circulating plating solution the required amounts of bath ingredients. This addition preferably is made by charging a filter, used in chemical reduction plating operations, with proper amounts of bath additives to maintain 15 the desired concentration.

20 Referring now more particularly to the accompanying drawing, which illustrates preferred apparatus comprising at least one plating tank, a heat exchanger, a filter and a pump connected in series, and control valves for carrying out the practice of the invention, articles which are to be coated with nickel or other metal are immersed in a 25 reduction plating solution in plating tanks indicated at 10 and 12. Although two tanks are illustrated, it will be understood, of course, that one or any number of tanks 30 may be employed, a plurality of tanks merely being connected in parallel, each in series with the heat exchanger, filter, and pump.

35 For proper deposition of nickel by chemical reduction plating, the temperature of the plating solution should be relatively high. Moreover, as mentioned above, in order to remove harmful ingredients either precipitated or mechanically dragged into the bath, the solution is continuously filtered. One of the most difficult problems 40 heretofore encountered has been that of precluding or minimizing the continued deposition of nickel or other metal as the hot plating solution is passed through the filter and other auxiliary equipment.

45 The practice of the present invention contemplates circulating plating solution, heated to the desired temperature in a conventional manner as by steam coils (not shown), through plating tanks 10 and 12, a heat exchanger 14, a fluid pump 16 and a filter 18 connected in series with said tanks, and withdrawing hot used plating solution from the plating tanks 10 and 12 through pipes 50 20 and 22, the flow being regulated by valves 24 and 26, and rapidly quench cooling the solution to a temperature at which plating does not occur. This is accomplished in the apparatus illustrated in the drawing by recycling cooled plating solution from the heat exchanger, having a 55 cooling fluid inlet 28 and outlet 30, by means of a pump 16, back through pipes 32, 34, 36 and 38, control valves 40, 42 and 58, to the heat exchanger where it mixes with the hot plating solution being withdrawn from the plating tanks through pipes 20 and 22 and serves to immediately 60 quench the hot plating solution to a lower temperature. In operation, the plating solution from the heat exchanger 14 may be continuously filtered by passing a portion of it through pipe 44 and filter 18 and recycling the remainder through the heat exchanger 14. If desired, a portion of the circulating bath can be simultaneously recycled to an addition tank 60 through pipe 46 and valve 48.

65 Although the quantities of solutions and flow rates thereof through pipes generally will be dictated primarily by the metal being deposited, the heat content of the solutions, the temperatures involved and the particular bath composition, in a particular instance excellent results have 70 been obtained by recycling approximately three times the

volume of hot plating solution continuously being removed from the plating tank. The temperature of the hot plating solution removed from the plating tanks, typically about 195° F., is thus quickly reduced to about 160° F. by mixing therewith three times its volume of cooled recirculated solution having a temperature of about 145° F. The 160° F. temperature is thereafter reduced to 145° F. by passing the solution through the heat exchanger, a portion of this effluent being passed to the filter and thence to the plating tank through valves 50, 52 and pipes 54 and 56 while the remainder is recycled by the pump 16 to the heat exchanger through pipe 38 and control valve 58 as described above.

The invention contemplates the use, preferably in combination with the aforementioned quench cooling of the hot used plating solution, the original bath makeup use of, or bath maintenance by, one or more water-insoluble salts of the metal to be deposited together with the appropriate reducing agent and/or other bath additives. In depositing nickel, for example, the proper plating solution concentrations preferably are maintained by addition of water-insoluble nickel salts. In practice, metal salts, as well as other bath ingredients, are added to the bath through an addition tank 60 where the resulting slurry, or solution in case it is desired to employ water-soluble salts, is pumped to the filter 18 and thence either back to the addition tank 60, having an outlet pipe 76 and control valve 78, or to the plating tanks 10 and 12.

Depending upon the particular type of filter employed it is desirable in many instances to employ a filter aid, such as finely divided asbestos or diatomaceous earth, in order to form a filterable cake. Such a filter aid can be added to the mixture in the addition tank 60 and thence pumped to the filter. In the drawing, the filter 18 is provided with a gas outlet 62 and control valve 61 to permit discharge of carbon dioxide or other gases formed during gradual dissolution of bath additives into the plating solution. To facilitate cleaning the filter a compressed air source (not shown) can be discharged through the filter 18 by means of valve 64 and inlet pipe 66, valve 68 permitting draining the apparatus when desired.

When water-insoluble salts of the metal to be deposited are used, a slurry is formed in the addition tank 60, valves 40 and 74 are either closed or adjusted to permit the desired flow and the slurry is pumped through valve 78 and pipe 76 to the filter 18 where it deposits over the filter media, formed typically of heat and chemical resistant cloth or fiber. If desired to build up a thicker coating on the filter media, valve 72 and valve 74 are closed and the solution is recycled back to the addition tank 60 through pipe 46 and valve 48. The plating solution being passed through the filter 18 gradually dissolves the metallic salts as the metal already in solution is depleted in the plating operation. Hence the procedure provides an extremely efficient method of controlling the plating operation and maintaining the proper bath concentration.

The present invention is particularly well adapted for use in the chemical reduction deposition of nickel. Typical of a nickel reduction plating bath which may be regulated in operation by the practice of the present invention is the following bath composition employing water-soluble nickel salts where the quantities expressed are per liter of water:

|                      |             |    |
|----------------------|-------------|----|
| Nickel chloride      | grams       | 30 |
| Sodium hypophosphite | do          | 10 |
| Glycollic acid (70%) | milliliters | 35 |
| Sodium hydroxide     | grams       | 15 |

It will be understood of course that the above bath composition is intended only as an illustration of a typical reduction plating bath and that the present invention is applicable to a wide range of nickel bath compositions. For example, plating baths containing about 5 to 50 grams per liter of a water-soluble nickel salt such as nickel

chloride, nickel acetate, nickel sulfate, etc.; approximately 5 to 100 grams per liter of a reducing agent, such as hypophosphorous acid, sodium hypophosphite or other soluble hypophosphites; and about 15 to 100 grams per liter of a buffer such as glycollic acid, sodium hydroxy acetate, sodium acetate, sodium citrate, etc. and/or other bath additives can similarly be replenished in accordance with the present invention.

It is to be understood that the present invention also 10 contemplates the formation of an improved nickel chemical reduction plating bath utilizing a water-insoluble nickel salt as an initial ingredient. Such a bath comprises an aqueous mixture of a reducing agent and a water-insoluble nickel salt selected from the group consisting 15 of oxy nickel salts such as nickel monoxide, nickel peroxide, nickel sesquioxide, nickelous nickelic oxide and nickelous superoxide; hydroxy nickel salts such as nickelic hydroxide and nickelous hydroxide; and nickel carbonates such as nickel carbonate and basic nickel carbonate. In 20 most instances it is desirable to additionally employ a buffer agent. A preferred bath of this type comprises nickel carbonate, sodium hypophosphite, and glycolic acid.

A bath of the above-mentioned type can be produced by dissolving the desired water-insoluble nickel salt or 25 salts in glycolic acid and thereafter adding the reducing agent. If another type buffer is used, for example, sodium acetate, sodium citrate or sodium hydroxy acetate, the nickel salt may first be dissolved in hypophosphorus or phosphorus acid, enough acid being used to obtain the 30 desired initial bath pH.

The following is an example of one reduction plating bath utilizing a water-insoluble nickel salt as an initial ingredient. The quantities expressed are per liter of water.

|                      |             |     |
|----------------------|-------------|-----|
| Nickel carbonate     | grams       | 15  |
| Glycollic acid (70%) | milliliters | 35  |
| Sodium hypophosphite | grams       | 10  |
| Preferred pH         |             | 5.0 |

A satisfactory range of ingredients comprises a mixture 40 of about 5 to 100 grams per liter of a water-insoluble nickel salt, approximately 15 to 100 grams per liter of a buffer such as glycollic acid, sodium hydroxy acetate, sodium acetate, sodium citrate, etc., and about 5 to 100 grams per liter of reducing agent such as sodium hypophosphite, hypophosphorous acid, or other hypophosphites.

We have discovered that excellent results are obtained 45 when the plating tanks, typically of steel or the like, are coated on the interior with porcelain or a heat resistant imprevious organic coating, a particular example being the commercially available phenolic coating known as "Heresite," a product of the Heresite & Chemical Co. Superior results have been obtained when the equipment coming in contact with the hot plating solution is formed 55 of tantalum which is extremely resistant to being coated by chemical reduction plating.

It is to be understood that, although the invention has 60 been described with specific reference to particular embodiments thereof, it is not to be so limited since changes and alterations therein may be made which are within the full intended scope of this invention as defined by the appended claims.

What is claimed is:

1. A method of depositing a metal from a chemical reduction type plating bath, said method comprising the steps of immersing an article to be coated into said plating bath which is maintained at an elevated temperature and is continuously recirculated through a filter, said plating bath being cooled just prior to passage through said 65 filter by mixture therewith of cooled plating solution.

2. In the deposition of nickel from a hot chemical reduction plating bath of the type comprising an aqueous solution of at least one nickel salt and a reducing agent in which said solution is continuously recirculated through 70 a filter to thereby remove harmful impurities, the improve- 75

ment which consists of precluding nickel deposition throughout the filter and associated apparatus as the plating solution circulates therethrough by passing the hot plating solution through a heat exchanger to cause said solution to cool, a portion of the cool plating solution from said heat exchanger being mixed with the hot plating solution as it is withdrawn from said both to thereby rapidly reduce the solution temperature below that temperature at which plating occurs.

3. Apparatus for chemical reduction plating operations, said apparatus comprising a plating tank, a heat exchanger and a filter connected in series by conduits to permit fluid flow from said tank through said heat exchanger and then through said filter and back to said tank, and means for recycling a portion of the fluid effluent of said heat exchanger to the inlet of said heat exchanger.

4. Apparatus for chemical reduction plating operations, said apparatus comprising a container for plating solution, a heat exchanger, a filter and a pump connected in series by conduits for the passage of said plating solution therebetween and valve means in said conduits to recirculate a portion of the heat exchanger effluent plating solution to the inlet of said heat exchanger.

5. Apparatus for carrying out chemical reduction plating operations, said apparatus comprising at least one plating tank, a heat exchanger, a filter and a fluid pump connected in series by conduits to permit fluid flow therebetween, said apparatus having control valve means for alternate and simultaneous filtering and recycling through said heat exchanger of a portion of said plating solution.

6. Apparatus for carrying out chemical reduction plating operations, said apparatus comprising a container for plating solution and a heat exchanger connected by conduits to permit fluid flow therebetween, means in said ap-

paratus for maintaining proper solution concentration, and means for recycling a portion of the heat exchanger effluent to the inlet of the heat exchanger.

7. In apparatus for use in chemical reduction plating operations, said apparatus comprising at least one container for plating solution, a heat exchanger, a filter and a pump, connected by conduits for series fluid flow, the improvement which comprises control valve and piping means adapted to withdraw a portion of cooled plating

10 solution from said heat exchanger and admix it with the plating solution passing from the container to heat exchanger.

8. Apparatus as set forth in claim 7 in which portions of the apparatus in contact with the plating solution are

15 formed of tantalum.

9. In a process for the deposition of nickel from a chemical reduction plating bath, said bath comprising an aqueous solution of at least one nickel salt and a reducing agent, the improvement which comprises withdrawing the

20 solution from said bath and passing it through a filter charged with at least one nickel salt to thereby replenish the nickel salt in said solution and simultaneously remove solid material from said solution, and then returning said

25 solution to said bath, said solution being rapidly cooled just prior to passage through said filter to a temperature below that at which plating occurs.

References Cited in the file of this patent

UNITED STATES PATENTS

|           |              |       |               |
|-----------|--------------|-------|---------------|
| 2,009,232 | Hood         | ----- | July 23, 1935 |
| 2,516,349 | Smith        | ----- | July 25, 1950 |
| 2,516,884 | Kyame        | ----- | Aug. 1, 1950  |
| 2,658,839 | Talmy et al. | ----- | Nov. 10, 1953 |